

Patented Jan. 15, 1924.

1,480,779

# UNITED STATES PATENT OFFICE.

ALADAR PACZ, OF CLEVELAND HEIGHTS, OHIO.

## COMPOSITION OF MATTER AND METHOD OF MAKING SAME.

No Drawing.

Application filed March 28, 1920. Serial No. 369,080.

To all whom it may concern:

Be it known that I, ALADAR PACZ, a citizen of the United States, residing at Cleveland Heights, in the county of Cuyahoga and State of Ohio, have invented a certain new and useful Improvement in Composition of Matter and Methods of Making Same, of which the following is a full, clear, and exact description.

10 This invention relates to the production of a finely divided metallic composition of which aluminum is the essential ingredient. Pure aluminum in the finely powdered state is a substance of great value and importance 15 in various technical uses, for example, in the production of high temperatures and the reduction of certain metals and alloys, and also in connection with the operation known as calorizing. According to the first 20 named use the powdered aluminum is mixed with a quantity of oxide of some metal or metals which aluminum will reduce, for example the oxide of iron or a metal similar to iron. Upon igniting the mixture, the 25 reaction proceeds very rapidly with the production of an extremely high temperature, much needed in certain welding operations. The result of this reaction is the reduction of the oxide to metallic form and the process 30 is often employed for the preparation of various metals and alloys, particularly the ferro-alloys, as well as the alloys of aluminum with silicon, etc. According to the second named use, the powdered aluminum is 35 introduced into a closed container in company with iron or steel articles and tumbled for several hours at a temperature around 900° C. in a hydrogen atmosphere, whereupon the aluminum alloys with the surface 40 of the ferrous metal in such wise as to protect the same in a very effective manner against oxidizing or corroding influences.

The preparation of such powdered aluminum has always been a matter of considerable difficulty. On account of its toughness, it has been found very difficult to cut the metal mechanically into pieces of sufficiently small size, while its great malleability has prevented the employment of any grinding 50 or crushing operations. It has been found possible by stirring the metal vigorously while cooling from a molten state to comminute it into small grains, and it is also possible by blowing a blast of air through a stream of the molten metal to atomize it into small particles, but in both cases the grains

are covered by a thin film of aluminum oxide. This oxide film renders it much more difficult to start the alumino-thermic reaction than it is in case the metal particles are 60 clean, and it impedes in a still more serious manner the process of calorizing.

The objects of my invention are the provision of a new, improved and simplified process whereby the necessary comminution 65 can be effected and with the production of grains which are preferably free from oxide coating; the provision of a powder which will react more quickly and easily for the production of heat or the reduction of metals 70 than the aluminum powders ordinarily used and also result in a superior product; the provision of a reacting material which shall produce a more fusible slag than heretofore; while further objects and advantages will 75 become apparent as the description proceeds.

The essence of my invention consists in alloying the aluminum with some substance which shall render it sufficiently brittle to enable its reduction to the powdered condition by mechanical means, and without injuring its reaction. Silicon is the substance which I preferably employ for this purpose in combination with the aluminum although other substances can be used in addition 80 thereto. When silicon alone is employed I preferably use an amount thereof equal to at least about 10 per cent of the resulting alloy, which causes the resulting alloy to become sufficiently brittle so that turnings 85 or borings of the same can be crushed in a ball mill much in the same way as cast iron borings. For reasons of economy and to avoid raising unduly the melting point of 90 the alloy I prefer to restrain the amount of silicon to the smallest amount that will afford the desired brittleness, although the proportion can be increased to any desired amount within the limits of practicable 95 fusion.

I find it perfectly feasible for many uses to alloy the aluminum with ferro-silicon rather than with pure silicon, preferably employing for the purpose a substance containing about 25 per cent of iron and 75 per cent of silicon. 10 per cent of this substance combined with aluminum results in a sufficiently brittle alloy for practical powdering, since the iron content itself has a considerable embrittling effect. Other metals can be added if desired such for example 105 as the various rare-earth metals for the pur-

pose of generating additional heat as set forth in my application filed March 19, 1920, Serial No. 367,085 or substances which shall be of assistance in chemical combination in the later use of the material, such as nickel or chromium in connection with the calorizing operation.

My improved alloy may be produced in any convenient manner, as by merely melting together the pure ingredients in an electric or other furnace, although I prefer to make it by the method described and claimed in my application filed March 18, 1920, Serial No. 366,968. The molten mixture is then preferably poured into a suitable mold and when cooled is turned into chips by suitable machinery, such as a boring mill, after which the chips are crushed or ground by any of the mechanical devices ordinarily used for such a purpose. However, the oxidation preventing quality of the silicon is such that the alloy can be blown if desired and the resulting grains will be oxide free; in this case, the silicon content can sometimes be reduced to a lower figure, say 5 per cent, the brittleness not being important but only the shielding quality of the silicon.

When employed in the welding operation, my improved material is superior to blown or stirred aluminum powder in that the reaction can be started more easily and yields an equally high temperature. When employed in the production of metals and alloys, the high temperature generated by the oxidation of the aluminum causes the silicon also to enter the reaction and assist the reduction thus serving the double purpose of producing a more fusible slag and more easily separable slag than is obtained when aluminum alone is employed (owing to the fact that the silica produced combines with the alumina to produce aluminum silicate which is much more fusible than pure alumina) and also prevents the contamination of the alloys by the aluminum. It is found that most alloys produced by the alumino-thermic reaction contain a quantity of aluminum as an impurity, some of the same becoming alloyed with the metal instead of assisting in the reaction, but my ex-

perience indicates that alloying of the aluminum is less likely to occur in case silicon be present and although a small amount of the silicon will sometimes become alloyed with the resulting metal, its presence is much less objectionable than that of aluminum. For use in calorizing, my improved powder operates much better than the blown or stirred aluminum powder owing to the absence of any superficial oxide, added to which the silicon is of independent advantage as a constituent of the coating. The adhesion of the coating and its chemical quality can also be enhanced by the use in the powder of small quantities of iron, nickel, chromium or the like alloyed with the aluminum. I do not restrict myself to the use of my improved composition of matter for the purposes herein mentioned but claim the same for all uses to which it may be applicable, and in general restrict myself in nowise except as specifically set forth in the annexed claims.

Having thus described my invention, what I claim is:—

1. A powdered alloy of aluminum and silicon containing at least about 5 per cent of silicon and the balance mostly aluminum.
2. A powdered composition of matter active alumino-thermically consisting essentially of aluminum alloyed with silicon, the amount of materials other than aluminum amounting to at least about 10 per cent and the silicon to at least about 8 per cent.
3. The process of producing an alumino-thermically active powder which consists in forming a brittle alloy of aluminum with one or more other metals, silicon being present, casting the same, making borings therefrom and crushing the borings.
4. The process of producing finely divided metallic particles containing aluminum as an essential constituent which contains the step of alloying the aluminum with at least about 5 per cent of silicon and subsequently reducing such alloy to powdered form in any of the modes heretofore employed in the case of pure aluminum.

In testimony whereof, I hereunto affix my signature.

ALADAR PACZ.